

# UNITED STATES PATENT OFFICE.

HANS KUŽEL, OF BADEN, AUSTRIA-HUNGARY.

## FILAMENT FOR ELECTRIC GLOW-LAMPS.

No. 914,354.

Specification of Letters Patent. Patented March 2, 1909.

Application filed March 23, 1906. Serial No. 307,695.

*To all whom it may concern:*

Be it known that I, HANS KUŽEL, a subject of the Emperor of Germany, residing at Baden, near Vienna, in the Empire of Austria-Hungary, have invented certain new and useful Improvements in Filaments for Electric Glow-Lamps, of which the following is a full, clear, and exact description, such as will enable others skilled in the art

10 to make and use the same.

My invention relates to filaments for electric glow lamps and has for its object a filament consisting of an alloy of antimony with one or more metals melting at very high temperatures, such metals as chromium, manganese, molybdenum, uranium, tungsten, vanadium, tantalum, niobium, titanium, thorium, zirconium, platinum, osmium or iridium. The alloys of the said 20 refractory metals and antimony not being directly obtainable by melting together their constituents and it being apparently impossible to make filaments of such alloys I shall first briefly set forth the method by which I 25 propose to make filaments, although this method forms a subject of other applications filed by me, namely Serial Nos. 239637 and 291909. According to this method filaments are made from plastic masses consisting of 30 colloids of the refractory metals with or without the addition of such refractory metals in a finely powdered solid state and with or without the addition of colloidal oxygen compounds of such refractory metals. The 35 plastic masses are then brought into the desired shape by any suitable process such as squirting, whereupon the threads or bodies thus obtained are dried and finally heated to a white heat in a neutral or reducing atmosphere. In order to manufacture filaments 40 of alloys of the said refractory metals and of antimony I incorporate into the plastic masses just described antimony either in a colloidal or finely powdered solid state. Or 45 instead of pure antimony I may incorporate

into the said plastic mass sulfur or oxygen compounds of antimony either in a colloidal or finely powdered solid state. In all cases I thus obtain a plastic mass containing besides the refractory elements also antimony. 50 This plastic mass is then in the manner above referred to brought into the desired form, then the bodies obtained are dried and finally heated to a white heat whereby the colloids are returned to their ordinary crystalline state, the oxygen or sulfur compounds being reduced at the same time in the reducing atmosphere. In any case I obtain by such heating filaments consisting of an alloy of the above named refractory 55 metals and antimony. The presence of antimony in the filaments has for its effect a notable increase of the electrical resistance of the filaments.

The oxygen or sulfur compounds of antimony, if any are used, should not exceed twenty per cent. by weight of the dry mass. The proportion of antimony in the finished filament is usually five to ten per cent. by weight of the entire filament, but it may increase even to twenty per cent. by weight without detriment.

I claim as my invention—

1. A filament for an electric glow lamp containing an alloy of a refractory metal as herein described with antimony.
2. A filament for an electric glow lamp consisting of an alloy of tungsten with antimony.
3. A filament for an electric glow lamp containing an alloy of tungsten with antimony.

In testimony whereof I have signed my name to this specification, in the presence of two subscribing witnesses.

HANS KUŽEL.

Witnesses:

JOHN GEORGE HARDY,  
ALVESTO S. HOQUE.